

1

3,042,505

## MULTI-FUNCTIONAL MIDDLE DISTILLATE ADDITIVE

William C. Hollyday, Jr., Plainfield, N.J., assignor to Esso Research and Engineering Company, a corporation of Delaware

No Drawing. Filed Oct. 18, 1960, Ser. No. 63,259

5 Claims. (Cl. 44—62)

The present invention is concerned with an improved multi-functional additive suitable for addition to middle distillates which will give these middle distillates improved pour, higher stabilities, higher detergencies and also improve the sludge characteristics. More particularly, the present invention relates to the preparation of improved low cold test hydrocarbon fuels, especially in heating oils and diesel fuels, kerosene, aviation turbo-jet fuels, and other fuels that are subject to low temperatures. In accordance with the present invention, an improved class of pour depressants is utilized with middle distillates which comprise condensation products of an acylated polystyrene with various amino compounds.

With the increase in the use of hydrocarbon fuels of all kinds, a serious problem has arisen in areas frequently subject to low temperatures in the cold test characteristics of fuels. Particularly, serious problems have been encountered by heating oils and diesel and jet fuels that have too high a pour point, resulting either in distributional or operating difficulties or both. For example, the distribution of heating oils by pumping or syphoning is rendered difficult or impossible at temperatures around or below the pour point of the oil. Furthermore, the flow of the oil at such temperatures through the filters cannot be maintained, leading to the failure of the equipment to operate.

It is well known to add pour depressants to lubricating oils to lower the pour point. These lube oil additives, mostly high molecular weight organic compositions formed by alkylation of benzene or naphthalene or derivatives thereof or by polymerization of lower molecular weight methacrylates, or by condensation polymerization of various kinds, are not satisfactory in service with middle distillate and lighter fuels. Poor performance of these additives might possibly result from the structural differences between waxes occurring in lubricating oils and so-called middle distillates.

A wide variety of compounds have been found to be effective as pour point depressants for lubricating oil. Among the best known are "Paraflow," "Santopour" and "Acryloid" and their modifications. They are prepared either by condensing aromatic compounds with long chain paraffins, such as wax, or by condensing olefinic esters. It is generally considered that these pour depressants are effective in that in cooling an additive-containing oil, the hydrocarbon chain of the additive becomes incorporated into the crystal lattice of the separated wax, while the other part of the pour depressant molecule prevents the crystals from adhering together to form a gel structure. The failure of these additives to be effective in middle distillates may at least in part be due to the basic difference in the composition between the wax in lubricating oils and that in middle distillate fuels.

It is, therefore, one object of the present invention to set forth an improved pour depressant for middle distillate and lighter fuels. The boiling ranges of these oils are generally about 250° to 750° F. Another object of the present invention is to use a multi-functional middle distillate additive for the improving of stabilization, the detergency, and the sludge characteristics of these fuels.

The petroleum distillate fuels in which the additive materials of the invention are employed consist of a major proportion, at least 95% of liquid hydrocarbons boil-

2

ing at temperatures between about 70° F. and about 750° F. These fuels include gasolines such as aviation, marine and automotive or motor gasolines, aviation turbo-jet fuels such as JP-1, JP-4 and JP-5 fuels, and diesel fuels such as marine, stationary and automotive diesel engine fuels.

Aviation turbo-jet fuel consists of at least 95% of a mixture of volatile hydrocarbons. It is defined by U.S. Military Specifications MIL-F-5616 and MIL-F-5624C. 10 Its volatility is such that its end point does not exceed 572° F. Its viscosity is between 0.5 and 1.5 centistokes at 100° F.

Diesel fuels as referred to in connection with the invention consist of at least 95% of a mixture of hydrocarbons boiling between 250° F. and 750° F. either by ASTM Method D 86-56 when their end points do not exceed 600° F. or by ASTM Method D-158-54. Diesel fuels are defined by ASTM Specification D-975-53T and fall into Grades 1D, 2D and 4D, in all of which the additive materials of the invention may be used. They have viscosities between 1.4 and 26.4 centistokes.

The liquid fuels in which the additive materials may be incorporated thus comprise at least 95% by weight of a mixture of hydrocarbons having a boiling range between 25 the limits of 75° F. and 750° F. and a viscosity between the limits of 0.264 and 26.4 centistokes at 100° F.

As pointed out heretofore, the new polymeric materials of the present invention giving improved pour, stabilization, detergency, and sludge dispersion characteristics 30 to a middle distillate fuel, are prepared by the condensation of acylated polystyrene with amino compounds.

The acylated polystyrene compounds are prepared with certain fatty acid chlorides of critical composition and are active pour depressants for middle distillates. The 35 acylates of interest have the following structure:



where the acyl group



is defined according to the "contributory number" table and R is normally a straight chain alkyl group of about 55 C<sub>7</sub> to C<sub>15</sub>, and X is a number from 3 to 20.

In general, the method of acylation may vary appreciably. The methods which are disclosed in U.S. Patent No. 2,703,817, entitled "Process for the Preparation of Lubricating Oil Additives," Inventor: George E. Serniuk, 60 and in U.S. Patent No. 2,500,082, entitled "Acylated Derivatives of High Molecular Weight Copolymers," Inventors: Eugene Lieber and William H. Smyers, may be utilized.

Broadly, the method of acylation comprises dissolving 65 the polystyrene in a suitable solvent, such as chlorobenzene, o-dichlorobenzene, or tetra chloro-ethylene and adding to the solution the equimolar carboxylic acid chloride/aluminum chloride complex at temperatures of 30° to 70° C. (preferably, 40° to 60° C.), with provision for 70 carrying away the evolved hydrogen chloride.

After all the acid chloride/aluminum chloride complex has been added (one mole per mole of phenyl groups in

the polystyrene, plus a slight excess) and hydrogen chloride evolution has stopped, the catalyst is destroyed with water or alcohol, the acylate is taken up in a suitable solvent, such as heptane or kerosene and washed with water and alkaline solutions. The resinous product may be isolated as the pure material by evaporating all solvents, or it may be used in solution for making blends in middle distillates.

For obtaining the superior acylated polystyrene, it is desired that the polystyrene starting material have an intrinsic viscosity within a range of about 0.2 to 2.0, preferably 0.8 to 1.5. These viscosities correspond to molecular weights within a range of from about 10,000 to 75,000, preferably 30,000 to 60,000 Staudinger (if the constant for isobutylene polymers is assumed to apply). Since the amounts of the other reactants are based on the weight of the polystyrene, the amount of polystyrene used will depend upon restrictions such as equipment capacity, etc. The cryoscopic molecular weight after acylation was about 700 to 5,000; the intrinsic viscosity about 0.05 to 0.5. The 700 molecular weight comprises, in essence, a trimer containing three acylated phenyl groups, whereas, the 5,000 molecular weight comprises, in essence, about 18 acylated phenyl groups, on the average, per polymer molecule.

The acylating agent chosen for the preparation of the acylated polystyrene of this invention will be aliphatic in nature and will preferably contain from 8 to 16 carbon atoms in a straight chain. Although  $C_8$ ,  $C_{10}$ ,  $C_{12}$ ,  $C_{14}$  and  $C_{16}$  acid chlorides are used in the examples specifically detailing the instant invention, any straight chain acid chlorides having the above requirements may be used. It is preferred that equimolar quantities of polystyrene and the acylating agent be used, however, from 0.80 to 1.20 mols of acylating agent per mol equivalent of polystyrene is operable. A large excess of acylating agent does not harm, but it does not react and so is wasted. As mentioned, suitable acyl groups include acetyl, butyryl, capryl, decanoyl, do-decanoyl, tetra-decanoyl, hexa-decanoyl stearoyl and benzoyl.

These acylates are condensed with primary and secondary aliphatic and aromatic amines such as methyl amine, n-propyl amine, t-butyl amine, n-octyl amine, n-do-decyl amine, n-octadecyl amine, aniline, N-methyl aniline, N-ethyl aniline, p-amino phenol, p-methoxy aniline, p-amino phenyl stearate, alpha-naphthylamine and beta-naphthylamine.

These compounds may be prepared in the following manner.

#### EXAMPLE 1



Simultaneous polymerization and acylation of polystyrene were carried out by the addition of a solution of 1.00 mole weight (104 g.) of polystyrene in o-dichlorobenzene solvent to an acid chloride/aluminum chloride complex. The complex contained 0.35 mole of n-dodecanoyl chloride, 0.35 mole of n-tetra-decanoyl chloride, 0.35 mole of n-decanoyl chloride and 1.05 moles of anhydrous aluminum chloride. The temperature was maintained at 5 to 40° C. during the reaction. The product was recovered by washing the reaction mixture with alkaline solutions and evaporating the solvent. The polymeric product had an intrinsic viscosity of 0.05 and was obtained in a yield of 96% of the theoretical, based on the assumption that the product contained one acyl group per phenyl group.

The acylated polystyrene prepared as described was dissolved in benzene and heated with one mole of do-decyl amine per mole weight of acyl groups. The tem-

perature was 100° C. and the catalyst a few pellets of sodium hydroxide. The following reaction took place:



Benzene and water were removed by distillation. The polymeric product contained 1.99% nitrogen, which indicates that about two-thirds of the acyl groups reacted with amine.

#### EXAMPLE 2

Various amounts of the pour depressants of the present invention were utilized in distillate fuels. A typical distillate fuel boiling in the range from 250° to 750° F. to which the present additives may be added are middle distillate heating oils. These fuels are of commercial grade and have typical properties as follows.

|    |                              |      |
|----|------------------------------|------|
| 25 | Composition:                 |      |
|    | Straight run gas oil         | 40   |
|    | Cat. cracked gas oil         | 60   |
| 25 | Inspections:                 |      |
|    | Gravity, °API                | 29.1 |
|    | ASTM, pour, °F., no additive | +20  |
|    | Flash Pensky-Martin, °F.     | 192  |
|    | Distillation ASTM, °F.—      |      |
| 30 | I.B.P.                       | 398  |
|    | 10%                          | 492  |
|    | 50%                          | 566  |
|    | 90%                          | 612  |
|    | F.B.P.                       | 644  |

35 The improvements obtained by adding the additives in accordance with the present invention are set forth in the following table. All pour points quoted hereafter were obtained by ASTM Method D-97-47.

The heating oil from Venezuela crude had a boiling range of 354-624° F., an API gravity of 37.6 and a viscosity of 2.35 cs. at 100° F. The heating oil from Canada crude had a boiling range of 316 to 685° F., an API gravity of 35.4, and a viscosity of 2.85 cs. at 100° F.

45 *Table I*  
POUR DEPRESSANT ACTIVITY OF ACYLATED POLYSTYRENE/AMINE CONDENSATE

| Test Oil Description             | Wt. percent Polymer <sup>1</sup> | Pour Point, °F. |
|----------------------------------|----------------------------------|-----------------|
| 50                               | 0.00                             | +10             |
| Heating Oil from Venezuela Crude | 0.01                             | -5              |
|                                  | 0.02                             | -5              |
|                                  | 0.03                             | -10             |
|                                  | 0.05                             | -15             |
|                                  | 0.10                             | -15             |
| 55                               | 0.00                             | +10             |
| Heating Oil from Canada Crude    | 0.01                             | 0               |
|                                  | 0.02                             | -10             |
|                                  | 0.03                             | -10             |
|                                  | 0.05                             | -35             |
|                                  | 0.10                             | -40             |

60 <sup>1</sup> Acylated polystyrene/amine condensate from Example 1.

#### EXAMPLE 3

In other tests, the effectiveness of the additives in controlling sediment were carried out. The results of these runs are shown in the following Table II. The heating oil used had a boiling range of 382-660° F., an API gravity of 35.0 and a viscosity of 3.10 cs. at 100° F.

70 *Table II*  
POTENTIAL SEDIMENT TEST

Test description: A sample of the middle distillate (200 ml.) is carefully filtered and then held at 210° F. for 16 hours, with exposure to air. During this treatment some sediment develops. This potential sediment is reported in mg. per 100 ml. of sample.

## Test results:

| Heating Oil Tested                                                                  | Pour Point, ° F. | Potential Sediment, mg./ml. |
|-------------------------------------------------------------------------------------|------------------|-----------------------------|
| (A) Mixed Heating Oil (50/50 cracked and straight run stocks from Venezuela crude.) | 0                | 0.45                        |
| (B) Same Heating Oil +0.02 Wt. percent product from Example 1-----                  | -20              | 0.10                        |

## EXAMPLE 4

In further tests, the effectiveness in the control of filter plugging were carried out with the following results shown in table III.

Table III

## ACCELERATED FILTER PLUGGING TEST

Test description: A sample of the middle distillate (5 gallons) is gradually raised from 75 to 235° F. over 16 hours. During this time sediment forms which is detected by filtering 12 liters of the sample. Demerits are assigned on the basis of the pressure drop across the filter element, the appearance (darkness) of the sediment removed from the filter sample, and the amount of sediment formed. If less than 12 liters of sample filter at a maximum pressure drop allowed by the conditions of the test, an additional demerit is involved.

## Test results:

| Heating Oil Tested | Liters of Sample Filtered | Demerits <sup>1</sup> |                     |                 |                  |
|--------------------|---------------------------|-----------------------|---------------------|-----------------|------------------|
|                    |                           | Pres. Drop            | Sediment Appearance | Sediment Weight | Overall (Aver.)  |
| (A) Table II-----  | 8.2                       | 8.5                   | 5.0                 | 3.8             | <sup>2</sup> 8.3 |
| (B) Table II-----  | 12.0                      | 4.4                   | 4.0                 | 3.7             | <sup>2</sup> 4.0 |

<sup>1</sup> Ranging from 0 to 10.

<sup>2</sup> Average demerit multiplied by the factor 12.0/8.2 because only 8.2 liters filtered.

<sup>3</sup> Equal to demerit obtained with commercial stabilizer.

The amount of the condensation product used may vary appreciably depending upon the particular stock in which it is used. However, the general range is from about 0.001 to 0.5 weight percent, preferably from 0.05 to 0.1%.

5 What is claimed is:

1. A petroleum distillate fuel composition having an improved pour and improved stability against sedimentation which comprises essentially a petroleum distillate fuel boiling in the range between 250° F. and about 750°

10 F. which has been improved with respect to pour point by the incorporation therein of a pour depressing effective amount in the range from about .001 to 0.5 wt. percent of a pour depressant which comprises essentially a condensation product of an acylated polystyrene and an amino compound, which condensation product has the following structure



20 25 wherein R is a straight chain alkyl group of about 7 to 15 carbon atoms, wherein x is a number from 3 to 20, and wherein R<sub>1</sub> is an amino group.

2. Composition as defined by claim 1 wherein said amino compound is a primary aliphatic amine.

3. Composition as defined by claim 1 wherein said amino compound comprises an aromatic amine.

4. Composition as defined by claim 1 wherein said amino compound comprises dodecylamine.

5. Composition as defined by claim 4 wherein the condensation product comprises about 1 mol of dodecylamine per mol of acyl groups.

## References Cited in the file of this patent

## UNITED STATES PATENTS

40 2,703,817 Serniuk ----- Mar. 8, 1955